

## UNITED STATES PATENT OFFICE

HARRY P. BANKS AND GLENN DAVIDSON, OF SEATTLE, WASHINGTON, ASSIGNEES TO  
I. F. LAUCKS INC., OF SEATTLE, WASHINGTON, A CORPORATION OF WASHINGTON

## PROCESS OF MAKING AN ADHESIVE AND THE PRODUCT THEREOF

No Drawing.

Application filed August 10, 1925. Serial No. 49,442.

Our invention relates to the process of making an adhesive and the product thereof. More particularly, our invention relates to the process of making an improved adhesive and to the product thereof by combining milk 5 casein and soya bean flour, or like vegetable protein, such as the protein of the peanut as it is contained in flour made from peanut cake or meal, and the protein in flour made from cottonseed cake or meal, and similar protein containing meals which when used in the same manner as is described for soya bean flour herein, react in similar manner and produce similar effects in the finished adhesive.

Our invention will be described in relation 15 to the particular problems obtaining in the manufacture of a suitable adhesive for ply wood panels. However, while our invention will be thus described in connection with the 20 particular problems of a particular use, nevertheless it is not to be deemed as limited to any such specific use, but is applicable to all uses where like problems and conditions obtain,—for example, in the manufacture of 25 sizings, calcimines, etc., where an efficient and relatively inexpensive adhesive is desired.

One of the definite conditions to be satisfied in providing an adhesive for ply woods is the providing of an adhesive which is characterized by the property of maintaining the 30 glue on the glue line in proper condition to form a bond. It will be remembered that in the making of ply wood after applying the adhesive to the cores or faces and assembling 35 of the same, the assembled panel is of necessity allowed to stand for a period of time because of plant requirements, until a full rack of panels is assembled and ready for the application of pressure. The problem is to 40 maintain the glue at such consistency that it will be held on the glue line in a proper degree of thickness to form said bond when pressure is applied.

Ordinary cold process glues are applied to 45 the veneer in the form of a sirupy colloidal

solution of the adhesive materials. Under ideal conditions, a certain time, dependent upon the nature of the glue, wood, etc., should be allowed to elapse before the two surfaces to be attached should be brought 50 into intimate contact by means of pressure. This period of time is referred to in literature concerning glueing as the "time of assembly". During this "time of assembly", the glue changes from a sirupy solution to a more or 55 less gelatinous film upon the surface of the wood. This is due, among other things, to loss of moisture from the glue to the wood upon which it is spread and to surrounding air. Now if pressure is applied before the 60 glue has attained this condition of a gelatinous film, i. e., while it is still in its original sirupy condition, the glue is comparatively easily forced out of the joint, e. g., in veneering out at the edges of the panel. It is also 65 under the above conditions relatively easily absorbed deeply into the pores of the wood, too far away from the glue line to be of service in enhancing the strength of the bond. The above conditions lead to what is termed 70 a "starved joint". A primary object of our invention is to provide a glue which will overcome to a certain extent this difficulty of starved joints encountered in veneering practice, where it is not possible to control the 75 time of assembly. That is, racks of panels must in practice be placed under pressure as rapidly as they can be assembled. Accordingly, the time which ordinarily elapses during the assembling and placing under pressure of a rack of panels gives a sufficient time 80 of assembly for the bottom panels in the rack, but frequently an insufficient time for the top panels, i. e., the last panels assembled. It is of course understood that the rack as a 85 whole cannot be allowed to stand to give sufficient time of assembly for the top panels, lest the glue on the bottom panels becomes entirely dry. Ordinarily milk casein formulæ give a sirup free from colloidal adsorbent 90

material and accordingly starved joint trouble is frequently aggravated with these glues. We have found it possible, however, to greatly reduce the tendency toward starved joints with milk casein glues by admixing with the milk casein, soya bean flour. The soya bean flour, being more difficultly dispersed than the milk casein, will partly disperse and partly remain as a flocculent adsorbent material floating in a milk casein dispersion when the mixture of milk casein and soya bean flour is treated with the ordinary reagents hereinafter mentioned for producing milk casein dispersion. This partially dispersed soya bean flour contributes to a certain extent in and of itself to strength of the bond formed between two surfaces of wood, but what is of greater importance, it appears to act as a sponge and prevent the escape of the glue from the glue line in cases where pressure is applied before sufficient time of assembly has elapsed as outlined above.

The term "partially dispersed soya bean flour" is used to designate the flour when part thereof has been broken up and subdivided to a degree of fineness required by colloidal dispersion, and part thereof still remains a flocculent adsorbent material.

The term "dispersion" is used here in the recognized sense developed in colloidal chemistry. Colloids or dispersed systems, can be formed in two different ways: (1) by subdividing coarse materials into fine particles, or (2) by gathering smaller particles or molecules or atoms together to a particle of the size of a colloidal particle. The first class we call "dispersion" methods and the second class "condensive" methods. Hence colloidal chemistry deals with the behavior and properties of matter in the colloidal condition, which, as we have seen, means a certain very fine state of subdivision, there being no sharp limitations to the size of particles in colloidal dispersion.

In connection with the problem of maintaining glue on the glue line, the following condition is to be noted. In the manufacture of ply wood, the plant may have the material from one log which is particularly free from resin, while the material from the next log may be very resinous. Therefore, there is this mixed product to be dealt with in manufacturing ply wood that cannot be foreseen. The resin seems to form a more or less smooth hard surface or coating, and this coating or film, so far as we are able to determine, seems to provide a body as it were which prevents the glue from gripping or taking hold of the fiber of the wood. The alkaline portion of the glue seems to cut this film and make it possible for the glue to act upon the fiber of the wood. Therefore, the importance of having a sufficiently active alkaline portion present in the glue is manifest. However, if

such excess active alkaline agent is present in milk casein glue, where the said glue is to be applied to materials relatively free from resin, then such alkaline agent seems to lower the adhesive properties of the milk casein element.

This results from excessive penetration in the wood of highly alkaline glue. Our aim is to provide an adhesive which overcomes these objections and is applicable to use upon both types of wood, that which is characterized by having excessive resin present and that which is relatively free from resin.

When the chemicals, that are usually added to milk casein to form glues, are used with a mixture of milk casein and soya bean flour, a certain amount of dispersion takes place, both of the milk casein and soya bean flour, or of the proteins of the soya bean. Our experience is that alkalinity chemically is necessary for this dispersion of the soya bean material. With most of the ordinary mixtures added to milk casein to form glue, alkalinity is developed; for example, lime plus either sodium fluoride, sodium phosphate, sodium borate, sodium silicate, and the like in water, form caustic soda,—these being the usual chemicals added to milk casein glues, i. e. these are the ordinary reagents for producing milk casein dispersion.

The milk casein, however, seems to have a further effect of acting like a protecting colloid on the partially dispersed soya bean material. For example, partially dispersed soya bean flour, while it has a certain amount of adhesiveness, does not form a smooth, easily spread glue. Be it noted by "smooth" is meant that the mass is free from lumps. Very finely ground milk casein is difficult to disperse in a liquid, because it is difficult to completely wet. The same is true in some instances of soya bean flour. Soya bean flour may be heat-treated, however, if desired, and among other results an increased ease of wetting may be provided of a soya bean flour before it is heat treated. On the other hand, more coarsely ground milk casein is comparatively easy to wet and this is also true of highly heat treated soya bean flour. Therefore, if it is desired to use finely ground milk casein, a ready dispersion may be attained by mixing with the milk casein a proper proportion of soya bean flour, which has received a high degree of heat treatment. "Coarse" casein may be defined, for purposes herein, as casein which would not pass a thirty-mesh screen, while "fine" casein may be defined as casein which would pass a sixty-mesh screen. Also, if it is desired in a certain formula to use soya bean flour, which has had little if any heat treatment, a ready dispersion may be greatly facilitated by addition of a proper proportion of coarsely ground milk casein. As respects the spreadability of the glue, it

should be noted that this feature is also an essential characteristic of a glue, particularly when used for ply wood. By this is meant that it may be mechanically applied by the 5 roller means to the core or to the face members constituting the ply wood structure. By adding milk casein to the soya bean flour, the mixture smooths out, and a great improvement is effected.

10 It is of course possible to treat soya bean flour without any such mixture of milk casein, so as to form a smooth easily spread glue, and the addition of milk casein, therefore, be it particularly noted, is only one means of 15 effecting the desired result of smoothness and spreadability.

Furthermore, our experience shows that the mixture of partially dispersed soya bean material makes an improvement on said 20 milk casein formulæ, especially such as tend to give a thin glue, in that the soya bean flour functions as an adsorbent. Of course, inert adsorbent materials may be added to such thin milk casein to function as an adsorbent, as is sometimes done by adding so-called "sander-dust," i. e., wood flour. By 25 adding to the milk casein a partially dispersed soya bean flour, which, even though partially dispersed, has in itself considerable adhesiveness, a great improvement is effected over simply the inert non-adhesive adsorbent. The excessive penetration of 30 highly alkaline glue, hereinabove referred to, may be off-set by "sponge" action of partially dispersed soya bean flour. The soya bean flour, however, does not prevent the alkaline portion of the glue cutting through the resin film on the surface.

40 The soya bean flour or like vegetable protein thus serves a double purpose. First, it acts as an adsorbent material for the milk casein, and, second, it has adhesive qualities in and of itself.

45 The proportions of each ingredient, milk casein, soya bean flour, or like protein material, may vary within wide limits. Where soya bean flour is desired to be the principal 50 ingredient, only enough milk casein is used to form a smooth glue, the milk casein acting as a protecting colloid. On the other hand, where it is desired to provide a glue which overcomes the objections above noted, 55 which obtain in milk casein formulæ, by furnishing an adsorbent property, a small amount of soya bean flour or like vegetable protein material may be added. The proportions may vary in the range from one- 60 tenth of one part milk casein to one part of soya bean flour to ten parts of milk casein to one part of soya bean flour. The particular definite proportions must be determined for the particular use for which the said product 65 is to be applied. Specific typical formulæ,

which we have developed, are noted as follows.

For ply wood purposes:

|                        | Parts | 70 |
|------------------------|-------|----|
| Soya bean flour        | 150   |    |
| Coarse milk casein     | 30    |    |
| Lime                   | 50    |    |
| Resin                  | 50    | 75 |
| Caustic soda           | 30    |    |
| Sodium silicate        | 90    |    |
| Potassium permanganate | 10    |    |
| Water                  | 790   |    |

|                     | Parts | 80 |
|---------------------|-------|----|
| Soya bean flour     | 150   |    |
| Coarse milk casein  | 50    |    |
| Magnesia            | 90    |    |
| Caustic soda        | 30    |    |
| Trisodium phosphate | 20    | 85 |
| Water               | 600   |    |

|                                       | Parts | 90 |
|---------------------------------------|-------|----|
| Fine milk casein                      | 80    |    |
| Soya bean flour                       | 20    |    |
| Lime                                  | 15    |    |
| Sodium fluoride                       | 12    |    |
| Water to bring to proper consistency. |       |    |

For sizing:

|                              | Parts | 95  |
|------------------------------|-------|-----|
| Soya bean flour              | 35    |     |
| Milk casein                  | 5     |     |
| Sodium fluoride              | 2½    |     |
| Lime                         | 2½    |     |
| Water to proper consistency. |       | 100 |

We have found that respecting soya bean flour or flour ground from soya bean cake, which is the residue remaining from the soya bean after a portion or all of the oil has been removed, certain new and useful properties are imparted to the soya bean flour by means of heat treatment of the same before it is admixed with the chemicals commonly used.

This part of our disclosure constitutes the 110 subject matter of a co-pending application, Serial No. 116,010.

We believe that such heat treatment causes 115 partial coagulation of the protein material, and, in fact, it is stated by other investigators of soya bean material that certain constituents of the soya bean protein are coagulated by heat, the amount of coagulation being dependent on the degree of heat and the duration of the heat.

It will be understood that in the milling of 120 soya beans to extract oil and make pressed cake, a certain amount of heat is used. The heating is in general by two different methods. In making the so-called round cake or "cartwheel" cake, the heating is with live steam on the crushed beans for about one minute, or at least for a very short period of time. In making the flat cake known as "English style cake" which is further exemplified as the standard product of the Anglo- 125

Chinese Eastern Trading Co. it is understood, the heating is accomplished by cooking the beans at a temperature slightly below the boiling point of water, (about 200° Fahrenheit), for an hour or more. In each case, after the heating process, the beans are placed in a suitable container and subjected to pressure to extract the oil and form the cake. It will be seen, therefore, that the beans are subjected to quite different treatments in the two processes which result in the two styles of cake. We find in practice that there is a great difference between the flours made from the two kinds of cake as far as their value and adaptability for making adhesives is concerned.

The so-called "cartwheel" cake of commerce is very irregular in quality and condition of protein and is quite liable to mold and still further impair its usefulness for adhesive purposes. This tendency to deteriorate in storage and during transportation is due in part at least to the high moisture content (15% to 17%). The "English style" cake, as described above, or the meal obtained by coarse grinding of same, however, is quite uniform in condition of the protein content, the moisture content is lower, being eight to ten per cent and oil content approximately six per cent. This cake keeps well in storage and during transportation. When "cake" is hereinafter noted in this application we refer to this "English style" pressed soya bean cake.

At times we find even this cake to have a degree of non-uniformity in condition of the protein due to a degree of heating of the beans or cake which is greater or less than the average. We find for example some cake that is in a condition that we call raw; it is to be understood, however, that what we term "raw cake" has nevertheless been subjected to the action of heat, and the protein constituents, as compared to those of raw beans, has, of course, been much changed or coagulated. However, we term flour from such cake "raw flour" to distinguish it from other flours which, as we can determine by tests, have been subjected to greater degrees of heat.

We have found that adhesives made from what we term "raw" flour are quite inferior. When the dry glue powder composed of such flour as a base, together with the other ingredients comprising the formula, is mixed with water the resulting glue or adhesive is very lumpy and hard or impossible to mix uniformly. At the same time it has a great tendency to foam considerably in mechanical mixers and spreaders. Foam, of course, ruins glue or at least greatly impairs the strength of the bond.

We have determined that if we start with raw flour which has the extremely undesirable properties described above and subject

such flour to heat, we then correct these defects and produce a flour which, when mixed in accordance with our regular formulæ set forth in the above named applications, will make a good adhesive or glue. The amount of heating to which the raw flour is subjected in such a process depends upon the degree of heating which the cake, from which the flour is made, has previously received. As this necessary heat treatment varies somewhat in amount or degree with different lots or shipments of flour received, we have contrived certain tests which we apply to the flour to determine its degree of "rawness." We then adjust the heat treatment, both as to degree of temperature and length of time, so as to produce flour containing protein coagulated to the proper degree.

One of the tests is what we term the absorption test: Twenty (20) grams of flour are mixed with twenty (20) grams of water and the mass kneaded into a small pat. This pat when so made must not be too sticky, but at the same time should have an appreciable degree of stickiness. As a measure of this stickiness we would say that it is just sufficient to pick up a fifty grams brass weight having an area of one square inch but it should not hold such weight for more than a few seconds. Also the mass is made into a round ball and dropped from a height of three feet to a wood surface. It should not flatten out to any extent but should keep its spherical shape and be practically on the point of showing a slight rebound. If the pat as above prepared will not pick up the weight, but is crumbly and mealy, then it is not raw enough for our purposes, i. e., it has been heated too much. If it is too sticky, then it is too raw. The pat test determines all heat up to the time of the expression of the oil and drying and milling and processing in the presence of live steam. If at the end of the processing, the pat test shows that it is too raw, then it is reheated to the requisite amount.

We are also able to judge as to the amount of heating to which a flour has been subjected and the further amount required by the smell, although this characteristic is very difficult to describe in words. The flour used in making the absorption or pat test above described has the "green" odor probably best described as suggesting new mown alfalfa hay. Heating makes this odor less pronounced and imparts a cooked odor.

Further, of course, as noted above, we are able to determine the state of the flour by the action of the glue mixture, made with the flour as a base, in the mechanical or hand mixers, i. e., whether it foams or not. If it foams considerably, then it is too raw, and more heat is applied.

As a specific example setting forth the steps

70

75

80

85

90

95

100

105

110

115

120

125

130

of the process of making and mixing an adhesive composition:

Mix dry in suitable batch mixer.

- 5 150 parts of soya bean flour
- 30 parts of coarse casein
- 50 parts of lime
- 50 parts of rosin
- 10 parts of potassium permanganate.
- 10 In suitable mixer place 600 parts of water, add the mixture of dry ingredients listed above. Stir until well mixed. Dissolve 30 parts of caustic soda in 60 parts of water and add to the glue mixture while stirring. Stir
- 15 for 10 minutes, add 90 parts of sodium silicate and 130 parts of water. Stir for five minutes. The adhesive is now ready for spreading in mechanical spreader on plywood. The characteristics of this adhesive, 20 the directions for mixing of which are given as one example, are described heretofore.

The adhesive embodying our invention is characterized by having the property of maintaining the glue on the glue line. Furthermore, the product is characterized by greater smoothness and spreadability and greater water resistance. Furthermore, the product thus provided has all the advantageous properties of straight milk casein for 25 mulæ adhesive, and at the same time overcomes the disadvantages inherent in milk casein glue, and said product is characterized at the same time by being much less expensive to manufacture than said milk casein 30 adhesive.

We claim:

- 1. In the method of making an adhesive, the step of adding to dispersed milk casein an adsorbent partially dispersed vegetable protein containing matter in the presence of water.
- 2. In the method of making an adhesive, the step of adding to milk casein dispersed in an aqueous alkaline medium a vegetable protein containing matter.
- 3. In the method of making an adhesive, the step of adding to milk casein dispersed in an aqueous alkaline medium soya bean flour.
- 4. In the method of making an adhesive, the step of partially dispersing vegetable protein containing matter in the presence of milk casein and water.
- 5. In the method of making an adhesive, the step of partially dispersing soya bean flour in the presence of dispersed milk casein and water.
- 6. In the method of making an adhesive, the step of heating soya bean flour and subsequently partially dispersing the same in an alkaline medium in the presence of dispersed milk casein.

- 7. In the method of making an adhesive, the steps of mixing soya bean flour, coarse milk casein, resin and potassium permanganate; adding water to the mixture thus

formed; stirring until well mixed; stirring in caustic soda dissolved in water and stirring in sodium silicate and water.

8. In the method of making adhesive, the step of adding soya bean flour to milk casein in the presence of lime and water and an alkaline metal salt which will form caustic soda in the presence of lime.

9. As an article of manufacture, an adhesive embodying milk casein, a vegetable protein containing matter, and water.

10. As an article of manufacture, an adhesive embodying milk casein, soya bean flour, and water.

11. As an article of manufacture, an adhesive embodying milk casein dispersed in an aqueous alkaline medium, and heat treated soya bean flour.

12. As an article of manufacture, an adhesive embodying milk casein dispersed in an aqueous alkaline medium, and steam treated soya bean flour.

13. As an article of manufacture, an adhesive embodying milk casein and vegetable protein containing matter, which constituents are intermixed in the presence of water in the range of proportions of one-tenth of one part milk casein to one part of said vegetable protein containing matter to ten parts of milk casein to one part of said vegetable protein containing matter.

14. As an article of manufacture, an adhesive embodying milk casein and soya bean flour, which constituents are intermixed in the presence of water in the range of proportions of one-tenth of one part of milk casein to one part of soya bean flour to ten parts of milk casein to one part of soya bean flour.

15. As an article of manufacture, an adhesive embodying milk casein dispersed in an aqueous alkaline medium and heat treated soya bean flour, which constituents are intermixed in the range of proportions of one-tenth of one part milk casein to one part soya bean flour to ten parts of milk casein to one part of soya bean flour.

16. As an article of manufacture, an adhesive embodying milk casein dispersed in an aqueous alkaline medium, and steam treated soya bean flour, either one of which constituents are intermixed in the range of proportions of one to one to ten.

17. An adhesive material comprising casein as a substantial ingredient together with a substantial amount of protein-rich seed meal incorporated with an alkaline earth oxide and a water-soluble alkali metal salt, which salt is capable of reacting in the presence of water with such alkaline earth oxide, and water in sufficient amount to produce a mixture of spreadable consistency.

18. An adhesive material comprising the reaction products of a substantial amount of casein, a substantial amount of protein-rich seed meal, an alkaline earth hydroxide, an

alkali metal compound of alkaline reaction, and water in sufficient amount to produce a mixture of spreadable consistency.

19. An adhesive material comprising the reaction products of a substantial amount of casein, a substantial amount of protein-rich seed meal, an alkaline earth hydroxide, an alkali metal hydroxide, and water in sufficient amount to produce a mixture of spreadable consistency.

20. An adhesive containing the reaction products of casein, soya bean meal and an alkaline earth oxide together with a water-soluble alkali metal salt which can react with alkali in the presence of water to form caustic alkali and a precipitate, the said salt and alkaline earth oxide being in amounts sufficient for the reaction products and water to dissolve the casein and the proteids in the soya bean meal, and water in sufficient amount to form an adhesive of the foregoing ingredients.

21. An adhesive material comprising the reaction products of a substantial amount of casein, a substantial amount of soya bean meal, an alkaline earth hydroxide, an alkali metal compound of alkaline reaction, and water in sufficient amount to produce a mixture of spreadable consistency.

22. An adhesive material comprising the reaction products of a substantial amount of casein, a substantial amount of soya bean meal, an alkaline earth hydroxide, an alkali metal hydroxide, and water in sufficient amount to produce a mixture of spreadable consistency.

In witness whereof, we hereunto subscribe our names this 3rd day of August, 1925.

HARRY P. BANKS.

GLENN DAVIDSON.

45

50

55

60

65